

No. 865,363.

PATENTED SEPT. 10, 1907.

C. F. DIECKMANN.

METHOD OF MAKING BIFOCAL LENSES.

APPLICATION FILED JULY 2, 1907.

Fig. 1.



Fig. 3.



Fig. 2.



Fig. 4.



Fig. 5.



Fig. 6.



Fig. 7.



Fig. 8.



Fig. 9.



Witnesses:

Frank S. Ober.

Waldo M. Chapin

Inventor  
Carl F. Dieckmann  
By his Attorneys  
Rosenbaum & Stockbridge

# UNITED STATES PATENT OFFICE.

CARL F. DIECKMANN, OF NEW YORK, N. Y., ASSIGNOR, BY MESNE ASSIGNMENTS, TO  
CRYPTOK COMPANY, A CORPORATION OF NEW YORK.

## METHOD OF MAKING BIFOCAL LENSES.

No. 865,363.

Specification of Letters Patent.

Patented Sept. 10, 1907.

Application filed July 2, 1907. Serial No. 381,894.

To all whom it may concern:

Be it known that I, CARL F. DIECKMANN, a citizen of the United States, residing at New York city, in the county of New York and State of New York, have invented certain new and useful Improvements in Methods of Making Bifocal Lenses, of which the following is a full, clear, and exact description.

My invention relates to the manufacture of bi-focal lenses, or the preparation of the blank therefor, and consists in the nature and sequence of the steps and operations by which separate properly formed pieces of glass of different indices of refraction may be perfectly welded or united together into a single, unitary or solid lens.

Lenses of the above character are now commonly manufactured in a number of different ways, but so far as I am aware, difficulty has been generally experienced by reason of gas, steam and air bubbles which are trapped between the surfaces of the separate pieces at the time they are welded. This difficulty probably arises on account of the hydroscopic nature of glass which attracts moisture to its surface from the air, and also the fact that all solid bodies carry on their surfaces a thin film of air which closely adheres thereto. The effect is particularly pronounced where the separate glass pieces are ground to the same curvature so that they fit closely when they are being welded. By the present invention this difficulty is overcome, and by the following steps and operations, particularly illustrated in the accompanying drawings, in which,

Figure 1 is a sectional view showing the glass pieces about to be assembled and welded. Fig. 2 is a similar view showing the same at the first stage of the operation. Fig. 3 is a top or plan view of the same. Fig. 4 illustrates the next stage of the operation. Figs. 5 and 6 show the two succeeding operations or stages. Fig. 7 shows one of the glass pieces having a slightly different shape. Fig. 8 shows the first step of my process as employed therewith. Fig. 9 illustrates a part used in this embodiment of the process.

Referring to the drawings in which like parts are designated by the same reference sign, A indicates a piece of glass for a lens and which may be termed the main blank or lens. B indicates another piece of glass of different index of refraction, and which may be termed the supplemental blank or lens. The blank A is first ground with a depression C, the curvature of which is suited to the requirements of the finished product, as hereinafter described. The blank B is superposed on the main blank A, but is not allowed to fit or rest closely thereon. The blank B is supported slightly away from the blank A at one or more points, which may be conveniently accomplished by the insertion of a small body D. In practice, I have employed a small bit of steel

for this purpose. The essential thing is to have the supplemental blank B held away from the main blank A at one or more points, and it is evident that this may be accomplished in any suitable manner.

The next step of the process is to apply heat to the assembled blanks so as to bring them to a welding temperature, or, more properly, a temperature at which they adhere, which is slightly below what is ordinarily known as a welding temperature. Under these circumstances, the blank B commences to merge into and adhere upon the surface of the blank A in the manner shown in Fig. 4. This welding action or adhesion occurs initially where there is contact between the glass pieces, and from this point or points the union spreads in the direction or directions of those points where the blanks are held apart, for example by the body or bodies D. Thus the union or adhesion spreads from a single point or points throughout the entire surfaces to be united, and ends at a predetermined or desired place where the surfaces were supported apart. The latter points are preferably near the circumferential edges of the parts to be joined, so that the gas, air and steam which is driven off by the heating is gradually crowded outward and away from the growing welded area, and the eventual total expulsion of such air and steam is absolutely insured. In other words, the position of the blanks to be joined, in accordance with the present invention, insures the commencement and the termination of the union or adhesion at such points or areas that there is always a vent for the gas, air and steam. The action is to have the area of union start at a single point of contact between the blanks, and constantly grow and enlarge from such point successively toward the circumferential point or points where the blanks are supported apart to form a vent, finally welding or uniting here also, after the gases are expelled and the blanks are united at every other point.

In Figs. 7 and 8, a supplemental blank B' is employed which is initially ground to conform to the curvature of the depression C. This is in some cases advantageous since it relieves this blank of the necessity of bending and conforming to a different shape. In this form of the invention the blanks may be supported apart by a circumferential ring E with a gap F through which the gases may escape. In this form of the invention, the welding or union obviously commences at the center and enlarges outward therefrom, instead of commencing at an eccentric or circumferential point and enlarging outward therefrom as with the first described embodiment of this invention.

The blanks or lenses being completely united in the manner shown in Fig. 5, it is merely necessary to grind and polish the resultant product into a solid lens as

shown in Fig. 6, and cut it into any desired form for eyeglasses or other purposes. The foreign body D, is ground away and eliminated in the grinding and shaping process.

5. What I claim is:

1. The process of welding or uniting together blanks for bi-focal lenses, which consists in supporting them in spaced apart relation by means independent of the blanks themselves and subjecting them to a welding or uniting temperature, whereby one of the blanks is caused to soften and settle down upon and adhere to the other.
- 10 2. The process of welding or uniting together blanks for bi-focal lenses, which consists in supporting them in spaced apart relation by an intermediate foreign body, and subjecting them to a welding or uniting temperature, whereby one of the blanks is caused to soften and settle down upon and adhere to the other.
- 15 3. The process of welding or uniting together blanks for bi-focal lenses, which consists in supporting them in spaced apart relation by an intermediate foreign body at the circumference of one of the blanks, and subjecting them to a welding or uniting temperature, whereby one of the blanks is caused to soften and settle down upon and adhere to the other.
- 20 4. The process of making bi-focal lenses, which consists in grinding a blank to form a depressed portion thereon, supporting a supplemental blank in spaced apart relation

therefrom at one or more points by means independent of the blanks themselves, and subjecting the blanks to a welding or uniting temperature whereby one of the blanks is caused to soften and settle down upon and adhere to the other, and grinding and polishing the resultant product.

5. The process of making bi-focal lenses, which consists in grinding a blank to form a depressed portion thereon, supporting a supplemental blank in spaced apart relation 35 therefrom at one or more points by an intermediate foreign body, subjecting the blanks to a welding or uniting temperature whereby one of the blanks is caused to soften and settle down upon and adhere to the other, and grinding and polishing the resultant product.

6. The process of welding or uniting together blanks for bifocal lenses, which consists in grinding a blank to form a depressed portion thereon, supporting a supplemental blank in spaced apart relation therefrom at one or more points near the circumference by an intermediate 45 foreign body, subjecting the blanks to a welding or uniting temperature, whereby one of the blanks is caused to soften and settle down upon and adhere to the other and grinding and polishing the resultant product.

In witness whereof, I subscribe my signature, in the 50 presence of two witnesses.

CARL F. DIECKMANN.

Witnesses:

CARL JUSSEN,  
GEO. E. KELLNER.